

Aug. 5, 1947.

A. J. MILLER ET AL

2,424,995

SELENIUM ELEMENT AND METHOD

Filed Nov. 5, 1942

*Fig. 1.*



*Fig. 2.*



INVENTORS  
ARTHUR J. MILLER  
OTTO J. MUELLER

BY

*D. G. Angus*  
ATTORNEY

## UNITED STATES PATENT OFFICE

2,424,995

## SELENIUM ELEMENT AND METHOD

Arthur J. Miller, Newark, and Otto J. Mueller, Rutherford, N. J., assignors to Federal Telephone & Radio Corporation, Newark, N. J., a corporation of Delaware

Application November 5, 1942, Serial No. 464,642

3 Claims. (Cl. 175—366)

1

This invention relates to selenium elements and particularly to a method of applying pressure against a selenium coated plate.

The object of the invention is to provide an arrangement whereby a selenium coating can be placed under a pressure without damage to the selenium.

In the making of selenium elements such as are used in dry selenium rectifiers one of the common steps in the process of making it is to apply a pressure against the selenium coating commonly placed upon a metallic base plate, usually at a raised temperature. It has been the experience in this art that most materials which are brought into contact with the selenium coating to apply the pressure are unsatisfactory, especially when the pressure is applied for a long time, owing mainly to the injury done to the selenium by their use. The restriction in the possible number of usable materials is probably due to the fact that a smooth surface must be brought against the selenium and also that whatever substance is used must be non-reactive or non-injurious to the selenium. A good grade of mica sheet has been found satisfactory for the purpose, but mica is expensive and not always easily obtainable in a satisfactory form.

In accordance with our present invention, we have discovered that an aluminum sheet can satisfactorily be pressed against the selenium if it is provided with a hydrated oxide coating of a rather critical quality. By the use of such an oxidized aluminum sheet it is possible to bring the sheet into high pressure contact with the selenium for a considerable period of time, such as a number of hours without injuring the selenium. We have found that if the oxide coating on the aluminum is too thin the selenium is injured or contaminated, apparently by reaction with the surface of the aluminum, and if on the other hand the coating is too thick the selenium tends to adhere to the aluminum more readily than to the base plate with consequent injury to the selenium surface. But by the use of a coating of the proper thickness and quality it is possible to apply a heavy pressure against the selenium and to heat treat it at the same time for a considerable time, if desired, and thus improve the characteristics of the selenium.

Our invention will be understood from the following detailed description and the accompanying drawing of which

Fig. 1 is a top view of a pressure device for compressing the selenium coated plate; and

Fig. 2 is a cross-sectional view in elevation of the arrangement.

2

In the drawing the disc 1 is a flat sheet which may be circular, preferably of steel and preferably also nickel coated and roughened in a well-known manner to receive a coating of selenium 2. The selenium coating may be applied in any well-known manner such as by placing selenium powder on the disc and then heating the disc to melt the powder and fuse it to the disc. The disc is shown with a centrally located hole 3 which is customarily used in order to build up a selenium element stack on a mandrel. Plates 4 and 5 represent the pressure plates of a press, the rest of the press mechanism not being illustrated. The plate or disc 6 is the aluminum disc 15 which has on it a coating of hydrated aluminum oxide 7 facing the selenium layer 2. When the pressure plates 4 and 5 are brought together the hydrated aluminum oxide coating is pressed firmly into contact with the selenium coated disc 20 and a pressure as high as many hundred pounds per square inch may be applied. At the same time a temperature may be applied if desired as by placing the compressed stack into an oven or if desired by applying a heating element to the 25 heads 4 and 5 of the press.

We have obtained a suitable aluminum oxide coating by anodizing an aluminum sheet. For the anodizing bath we have found that a sulphuric acid solution with a concentration of about 10% 30 by weight sulphuric acid is satisfactory, and that the cathode may for example be of copper, the anode being the aluminum disc or plate which is to be coated with the oxide. We maintain the temperature of the solution preferably at approximately 20° C. We apply a D. C. voltage to the anode and cathode and adjust the flow of current through the solution to be sufficient to establish an anodizing action. We have found that a current density of about 16.5 amperes per 35 square foot of aluminum surface area to be coated is satisfactory, although we have discovered that this can be varied within fairly wide limits, such as from about 4 to 32 amperes per square foot; and we allow this current to flow for about 40 seventeen minutes at this rate. While the current density to be used is not very critical so long as it is sufficient for the anodizing, the concentration of the solution in combination with the time of anodizing is of importance in determining 45 the quality of the coating. If it is not desired to coat the back of the aluminum disc, the coating on the back may be prevented as by covering the back with a material which will not coat, such as styrene. 50 Although the values of the solution concentration and the current flow and time of plating

given in the above method of anodizing the aluminum may vary to some extent, we have found that a serious departure from the directions given above will create a coating of aluminum oxide sufficiently different from the desired coating to produce trouble when used as a pressure contact plate over a considerable period of time.

In cases where the pressure is to be applied against the selenium surface for relatively short periods of time, thinner oxide coatings than those obtained by the above procedure may be found satisfactory enough. In cases where such thinner coatings may be used the thinner coatings may be obtained by the same anodizing process as described above except that the time of the anodizing in the solution may be made shorter or the current density may be made less.

What is claimed is:

1. The method of treating a selenium coated plate which includes pressing against the top surface of the selenium coating a hydrated oxide coated aluminum sheet, the thickness of the oxide coating being in the order of that obtained by anodizing the aluminum surface in approximately 10% by weight sulphuric acid solution for about seventeen minutes with a current density between about 4 and 32 amperes per square foot of aluminum surface to be coated.

2. The method of treating a selenium coated plate which includes pressing against the top surface of the selenium coating a hydrated oxide coated aluminum sheet, the thickness of the oxide

coating being in the order of that obtained by anodizing the aluminum surface in an approximately 10% by weight sulphuric acid solution for about seventeen minutes with a current density of about 16.5 amperes per square foot of aluminum surface to be coated.

3. The method of compressing a selenium coated plate which includes placing the plate between the pressure heads of a press with a hydrated aluminum oxide coated aluminum sheet in contact with the top surface of the selenium coating, said hydrated aluminum oxide coated sheet formed by anodizing the aluminum surface in approximately 10% by weight sulphuric acid solution for about seventeen minutes with a current density sufficient for anodizing.

ARTHUR J. MILLER.  
OTTO J. MUELLER.

#### REFERENCES CITED

The following references are of record in the file of this patent:

#### UNITED STATES PATENTS

| 25 | Number    | Name    | Date          |
|----|-----------|---------|---------------|
|    | 2,203,328 | Geisler | June 4, 1940  |
|    | 2,221,596 | Lorenz  | Nov. 12, 1940 |

#### OTHER REFERENCES

Anodic Coating of Aluminum, J. D. Edwards, published 1939, Trans Electrochemical Society, vol. 79, pp. 137-144.